

## UNITED STATES PATENT OFFICE

2,388,128

## ALLOY STEEL

Joseph C. Eckel, Ingram, Pa.

No Drawing. Application February 11, 1944.  
Serial No. 521,996

2 Claims. (Cl. 148—31)

A continuous search for steels with increasing mechanical properties, mostly those combining a high yield strength with a sufficient elongation, conducted through years definitely indicated the lack of such steels in the range of presently known low-carbon medium-alloy steels, most commonly employed for structural purposes. While both high strength and high elongation are frequently and conveniently produced in the high-carbon metals of this class by specific means, no method or composition of the steel known heretofore permitted to combine them in low-carbon steels of this type without resorting to a greatly increased alloy content. It can be said without the danger of contradiction that only steels of the stainless group, more specifically those possessing an austenitic structure, typified by the analysis of 18 per cent chromium and 8 per cent nickel, permitted the combination of these desired properties following manufacturing processes suitable for industrial production.

The present invention relates to a group of substantially corrosion and heat resistant steels belonging to the low-carbon medium-alloy type, the properties of which, after commercial treatment show a combination of heretofore unavailable unusually high yield point with an elongation assuring their value as an engineering material, and more particularly to steels containing about 0.10 per cent carbon, about 5 per cent nickel, about 2 per cent silicon and about 2.5 per cent chromium, permitting the replacement of comparatively expensive stainless steels for many applications where the mechanical properties occupy the pre-eminent position.

High-carbon medium-alloy group of steels offers a wide range of physical properties, combining high tensile strength with pronounced elongation, desired impact characteristics, and proper resistance to the notch effect on loading. Their desirable characteristics are largely a function of their carbon content. The alloying elements cannot be considered here as a direct cause of the properties of steel. On this account, in order to obtain the required mechanical properties following a predetermined heat treatment, the common practice for this group of alloys is to increase their carbon content to the range adequate for producing the desired results, either by incorporating this element into the body of steel during the process of its manufacture, or artificially building carbon content at the surface of articles by carburizing or similar processes.

Being amply capable of meeting mechanical requirements presented to this group of alloys, these steels possess, however, a decided negative feature associated with pronounced metallurgical changes occurring on heating high carbon steels containing a comparatively high alloy percentage in the process of their final assembly into fin-

ished products. These changes of properties are particularly pronounced in welding them. Heating involved in the latter brings the alloys to temperatures much higher than their upper critical point, and, unless proper precautions are exerted in order to prevent rapid cooling caused by the surrounding cold metal, there is always a possibility that the metal present in austenitic state might be transformed here into martensite or its decomposition products associated with low ductility and excessive hardness. A steel capable of meeting the severe treatment of the welding operation should have, therefore, a composition, in which carbon, usually considered as the most prominent component from the standpoint of welding characteristics, is reduced to a minimum consistent with an adequate mechanical performance of the alloy. The reduction of carbon content to the lowest possible percentage is, therefore, one of the objects of my invention.

The steels of my invention are addressed particularly to applications in which a high mechanical strength, an adequate ductility, good forming characteristics, freedom from welding trouble, and a reasonably good corrosion and heat resistance are combined, going hand in hand with reasonably simple processes of steel making, comparatively low costs, and freedom from complicated heat treating methods to be applied to the finished products.

Aviation and automotive industries and building of mobile equipment appear to be the natural field for steels having these qualifications, particularly when applied to parts of aircraft or automobiles, in which large surfaces possessing an elevated strength and resistance to atmospheric conditions must be produced. The steels of my invention are primarily suitable for the production of sheets, strip, and similar flat objects eventually fabricated either by forming or welding, or a combination of the two, into structural members of the character described.

I have found that steels containing 0.05% to 0.15% carbon, 0.30% to 0.65% manganese, 0.050% maximum phosphorus, 0.050% maximum sulphur, 0.50% to 2.00% silicon, 0.20% maximum copper, 4% to 6% nickel, and 2% to 6% chromium meet the above requirements in a particularly satisfactory manner. These steels respond to the commonly used heat treatment with readiness and completeness, permitting a wide range of properties, in which adequate yield point is combined with a sufficiently high elongation, and, which show, furthermore, a very important property of being hardened to a very high extent by application of cold working operations such as cold forming, retaining after the latter a sufficient degree of ductility to permit their application for structural purposes without incurring the danger of a sudden failure in use. This fea-

ture makes them particularly suitable for the manufacture of sheets and other flat products, in which the degree of cold drawing can be regulated at will and extended to the limit assuring the desired strength.

In order to illustrate the mechanical characteristics of the steels constituting the present invention and their response both to hot rolling and cold rolling, the following tabulation is given in the way of an example, but by no means limiting the scope of the present invention. Specimens represented in the tabulation, given below were made from a steel containing 0.08% carbon, 0.48% manganese, 0.008% phosphorus, 0.020% sulphur, 1.79% silicon, 0.02% copper, 15 4.94% nickel and 2.92% chromium, cast and rolled in a manner common to steel mill practices:

5 a low temperature drawing. In this case, more vigorous quenching in water resulted after a 700° draw in an elongation of 8%, while a somewhat milder quenching, from the same temperature in oil, resulted in a 6.5% elongation. This observation shows that the steel has tendency to remain austenitic after a reasonably vigorous quenching, which serves as a contributing factor to the pronounced increase of its strength by cold rolling. Better properties can be expected in this case, therefore, when a cold reduction operation of a sufficient intensity is used either alone or in combination with an appropriate stress relieving heat treatment, such as a low-temperature annealing.

10 15 The above tabulation, illustrating the mechanical properties of the steel constituting the subject of the present invention, indicates that they

| Gauge                                              | Treatment                    | Hardness, Rockwell B | Yield strength (0.2% offset) lbs./in. <sup>2</sup> | Tensile strength, lbs./in. <sup>2</sup> | Elong. percent in 2" |
|----------------------------------------------------|------------------------------|----------------------|----------------------------------------------------|-----------------------------------------|----------------------|
| <b>HOT ROLLED SHEETS</b>                           |                              |                      |                                                    |                                         |                      |
| 0.087"                                             | Hot rolled.....              | 111                  | 160,300                                            | 193,200                                 | 9                    |
| 0.035                                              | Cold reduced.....            | 115                  | 242,750                                            | 251,000                                 | 3                    |
| <b>HOT ROLLED, PICKLED AND COLD REDUCED SHEETS</b> |                              |                      |                                                    |                                         |                      |
| 0.035                                              | Box annealed at 1250° F..... | 99                   | 110,900                                            | 116,300                                 | 19                   |
|                                                    | Water quenched.....          | 110                  | 163,400                                            | 208,500                                 | 6                    |
|                                                    | Oil quenched.....            | 105                  | 168,600                                            | 199,200                                 | 6.5                  |
|                                                    | Water quenched:              |                      |                                                    |                                         |                      |
|                                                    | Drawn at 700° F.....         | 103                  | 177,800                                            | 195,300                                 | 8                    |
|                                                    | Drawn at 900.....            | 105                  | 194,000                                            | 199,200                                 | 4.5                  |
|                                                    | Drawn at 1000.....           | 103                  | 137,100                                            | 143,200                                 | 11                   |
|                                                    | Drawn at 1100.....           | 98                   | 120,300                                            | 128,400                                 | 14                   |
|                                                    | Drawn at 1200.....           | 94                   | 193,300                                            | 126,300                                 | 15                   |
|                                                    | Oil quenched:                |                      |                                                    |                                         |                      |
|                                                    | Drawn at 700° F.....         | 103                  | 179,200                                            | 194,800                                 | 6.5                  |
|                                                    | Drawn at 900.....            | 103                  | 155,400                                            | 158,000                                 | 6.0                  |
|                                                    | Drawn at 1000.....           | 102                  | 134,100                                            | 138,800                                 | 12                   |
|                                                    | Drawn at 1100.....           | 97                   | 120,800                                            | 129,000                                 | 16                   |
|                                                    | Drawn at 1200.....           | 95                   | 100,200                                            | 129,200                                 | 16                   |

An examination of these figures clearly shows that the steel has a very high yield strength together with an adequate elongation, even in a hot-rolled state, and that mill practices (particularly heating for rolling, finishing temperatures and piling or coiling temperatures) and finishing gauge have some effect on the finished hot rolled product. A combination of hot rolling with cold reduction, somewhat increasing the hardness of steel, leads to a really remarkable increase of the yield point, reaching 240,000 pounds per square inch, while the elongation remains as high as 3%. The usual heat treatment for uniform transverse and longitudinal properties, namely, quenching followed by a drawing operation, leads to the results expected in the steels of this type, namely, a gradual reduction in elongation. Among the above treatments, particularly interesting is water or oil quenching from above the critical temperature followed by

45 are much higher than the corresponding properties of the class of steels well known to the trade under the name of "low-alloy, high tensile-strength steels." This difference seems to be more of an average character than when specific treatments of selected steels are compared with certain values taken from the above tabulation.

50 A further advantage of steels proposed by me, which belong preferably to the fine grain fully killed type, containing a comparatively high percentage of nickel, is their marked resistance to the notch effect, particularly at low temperatures. This property commands the greatest interest in application of the steel to the aircraft construction, where the conditions are conducive to the greatest demand for this property. Furthermore, 55 their elongation and mechanical properties other than impact strength are but little affected by the lowering of temperature, as can be seen from the following table of properties obtained with 0.035" sheets:

|                                          | Yield strength (0.2% offset) |         | Tensile strength lbs./in. <sup>2</sup> |         | Elongation percent in 2" |        |
|------------------------------------------|------------------------------|---------|----------------------------------------|---------|--------------------------|--------|
|                                          | Room t°                      | 70° F.  | Room t°                                | 70° F.  | Room t°                  | 70° F. |
| Normalized from 1600° F.....             | 165,000                      | 183,600 | 192,200                                | 203,500 | 6                        | 6      |
| Water quenched and drawn at 600° F.....  | 180,800                      | 188,400 | 189,500                                | 203,500 | 7                        | 6      |
| Water quenched and drawn at 1200° F..... | 104,900                      | 121,600 | 124,000                                | 140,200 | 16                       | 15     |

When it is recalled that welding characteristics of most steels are largely a function of their carbon content, and when it is realized that the carbon content of the proposed steel is well below the content of this element of all medium alloy structural steels having the desired strength, better welding characteristics of the steels of my invention could be predicted in advance. This contention was amply supported by a comprehensive series of actual welding tests conducted principally with the use of the spot welding practice and which conclusively demonstrated the suitability of the selected carbon range in combination with the properly adjusted alloy content for welding applications. No pronounced hardening of the welds or areas adjoining them could be noted in specimens examined, and the welds were perfectly sound.

In applications involving high-strength thin structural members, such as used in construction of aircraft, any potential reduction of their thickness by corrosion plays a very important role in the selection of the material suitable for the purpose. On this account, the corrosion resistance of the proposed steels is of a very great importance to their potential users. It has been found that steels of the type proposed in the present invention have a practically seven-fold resistance than of plain carbon steel to the corrosion in industrial atmosphere taking place in the course of a five year exposure. The corrosion curve, expressing this property as a loss of weight per unit of area, is free from any unusual deviation from the shape of the curve which might be considered as a standard, differing from the latter only in the coefficient involved. Being pronouncedly superior from the corrosion resistant standpoint to the common carbon steel, the proposed steels have better corrosion properties than many proprietary alloys of low-alloy high-strength class sold at present, partially on the corrosion-resistance basis. Both in industrial atmosphere and in a stream of fresh water, specimens of the steels made according to my invention have the corrosion resistance about twice as high as some of the best known alloys of the above group.

The steel of the present invention has high strength and ductility, high resistance to impact, effective resistance to corroding media, and low 50

hardening capacity, so that it may be subjected to the usual operations incident to hot and cold forming and welding without sufficient hardening and subsequent loss of ductility to require heat treatment prior to structural application.

Though the steels of my invention are not intended for use as scaling-resistant material, their capability to withstand heat under oxidizing conditions is much greater than that of common carbon steels, in many occasions approaching that of so-called stainless steels, particularly in the lower temperature ranges. It is particularly worthy of attention to note the character of the scale formed. When a common carbon steel is subjected to the effect of temperature under a parallel set of conditions, the scale produced on it is of a loose type poorly adhering to the base and capable of being easily dislodged even by such mild agents as a stream of air. The scale formed on the steel of the present invention does not develop any loosely adhering layers of oxide. The oxide in this case is somewhat crystalline, tightly adherent, thin, and can be removed by mechanical means only with a considerable difficulty, offering a very adequate material for heat screens and similar applications, in which scaling resistance of high-cost stainless steels is superfluous, but the capability of resisting oxidation of common steels is not high enough to meet the requirements.

The present invention is not limited to the proportions set forth in the illustrative embodiments, but may be otherwise modified within the scope of the following claims.

35 I claim:

1. A severely cold worked shape of an alloy steel composed of 0.05% to 0.15% carbon, 0.30% to 0.65% manganese, 0.05% maximum phosphorus, 0.05% maximum sulphur, 0.50% to 2.00% silicon, 0.20% maximum copper, 4% to 6% nickel, 2% to 6% chromium, the balance being substantially all iron.

2. A severely cold worked shape of an alloy steel composed of 0.05% to 0.10% carbon, 0.35% to 0.50% manganese, 0.03% maximum phosphorus, 0.05% maximum sulphur, 1.75% to 2.00% silicon, 0.10% maximum copper, 4% to 6% nickel, 2% to 3% chromium, the balance being substantially all iron.

JOSEPH C. ECKEL.